

## UNITED STATES PATENT OFFICE

2,683,083

N-ALKYL-N'-(p-HYDROXYPHENYL) UREAS  
AS ANTIOXIDANTS FOR PETROLEUM HYDROCARBON FUELS

Eugene F. Hill, Detroit, and David O. De Free, Royal Oak, Mich., assignors to Ethyl Corporation, New York, N. Y., a corporation of Delaware

No Drawing. Original application December 9, 1950, Serial No. 200,112. Divided and this application July 26, 1952, Serial No. 301,167.

8 Claims. (Cl. 44—71)

1

This invention relates to new urea derivatives. More particularly our invention relates to N-alkyl-N'-hydroxyphenyl ureas. This application is a division of co-pending application, Serial No. 200,112, filed December 9, 1950, now abandoned, and a continuation-in-part of application Serial Number 200,115, filed December 9, 1950.

The substance N-p-hydroxyphenyl urea, has been described heretofore. This material possesses no utility in the field of oxidation inhibition. We have discovered, however, that by substituting the free amine of N-p-hydroxyphenyl urea with an alkyl group we obtain a class of substances which are powerful gasoline antioxidants. So far as we are aware it has not previously been known that the mere addition of an alkyl group to an otherwise inactive compound would produce thereby a material which would prevent deterioration of petroleum hydrocarbons by the action of oxygen.

Therefore it is an object of our invention to provide a new class of antioxidant materials useful in protecting petroleum hydrocarbons from deterioration in the presence of oxygen or air. In particular it is an object of our invention to provide a new class of materials which prevent the deterioration of motor fuels by oxygen.

In accordance with our invention we provide new ureas which contain the structure



wherein R is an alkyl group. By the term "alkyl" we mean saturated, straight, or branched chain or cyclic aliphatic hydrocarbon radicals. Examples of such alkyl radicals include methyl, ethyl, propyl, n-octadecyl, isopropyl, isobutyl, sec-butyl, 2-methylhexyl, cyclohexyl, methylcyclohexyl,  $\beta$ -cyclohexylethyl, etc.

The free amine from which our compounds may be considered as being derived, in addition to being inactive as an antioxidant, possesses a low degree of solubility in petroleum hydrocarbons. However, by substituting an alkyl group on the free amine nitrogen, in accordance with our invention, we not only increase the solubility in petroleum hydrocarbons but obtain the unexpected result that we thereby create an antioxidant material which is as potent as many commercial antioxidants and more potent than several.

As examples of the alkyl groups which can be

2

substituted in accordance with our invention we include methyl, ethyl, n-propyl, isopropyl, and the various isomeric butyl, amyl, and octyl radicals. However, we find that we can increase the alkyl chain beyond the limits enumerated above without impairing the antioxidant qualities of our invention. For example, when the alkyl group is as high as dodecyl or even octadecyl we still obtain extremely active antioxidant materials. As further examples of the alkyl groups which we can substitute in the compounds of our invention we include cyclohexyl and hydrocarbon substituted cyclohexyl radicals, as well as aralkyl radicals such as, for example, benzyl and hydrocarbon substituted benzyl radicals.

In general the compounds of our invention are prepared readily and in good yield by treating alkylisocyanates with p-aminophenol. In the examples which follow we illustrate the preparation of specific examples of the novel compounds of our invention, and in these examples all parts and percentages are by weight.

## EXAMPLE I

25 *N-n-propyl-N'-(p-hydroxyphenyl) urea.*—To a vessel provided with an agitator, means for returning reflux to the reaction vessel, means for introducing liquid reactants, and means for supplying heat was added 100 parts of p-aminophenol and 300 parts of toluene. This mixture was heated to a temperature of 50° C. and 85 parts of n-propylisocyanate was added over a period of one and one-quarter hours. At the end of the addition the mixture was heated for an additional period of 30 minutes. The reaction mixture containing the product as a suspended solid was filtered and the *N-(n-propyl)-N'-(p-hydroxyphenyl) urea*, 130 parts, was recovered in 67 per cent yield based upon the p-aminophenol employed.

## EXAMPLE II

30 *N-cyclohexyl-N'-(p-hydroxyphenyl) urea.*—In accordance with the procedure of Example I, 100 parts of p-aminophenol in 300 parts of toluene was treated with 113 parts of cyclohexylisocyanate to produce *N-cyclohexyl-N'-(p-hydroxyphenyl) urea*. This product had a melting point of 210° C.

## EXAMPLE III

35 *N-(mixed-amyl)-N'-(p-hydroxyphenyl) urea.*—In accordance with the procedure of Example I, 100 parts of p-aminophenol in 300 parts of toluene was treated with 101 parts of (mixed)

amylisocyanates to produce N-(mixed-amyl)-N'-(p-hydroxyphenyl)urea. This product had a melting point of 180° C. with decomposition.

#### EXAMPLE IV

*N-n-octyl-N'-(p-hydroxyphenyl)urea.*—In accordance with the procedure of Example I, 100 parts of p-aminophenol in 300 parts of toluene was treated with 142 parts of n-octylisocyanate. This product, N-n-octyl-N'-(p-hydroxyphenyl)-urea, had a melting point of 131° C.

#### EXAMPLE V

*N-n-butyl-N'-(p-hydroxyphenyl)urea.*—In accordance with the procedure of Example I, 100 parts of p-aminophenol in 300 parts of toluene was treated with 99 parts of n-butylisocyanate to produce N-n-butyl-N'-(p-hydroxyphenyl)-urea having a melting point of 158° C.

#### EXAMPLE VI

*N-n-dodecyl-N'-(p-hydroxyphenyl)urea.*—In accordance with the procedure of Example I, 100 parts of p-aminophenol in 300 parts of toluene was treated with 188 parts of dodecylisocyanate to produce N-n-dodecyl-N'-(p-hydroxyphenyl)urea having a melting point of 142° C.

The compounds of our invention are excellent antioxidants and we have illustrated this property in the table, wherein we have listed the results obtained by determining the oxidation stability of gasoline according to the Induction Period Method, ASTM designation: D525—46, as fully described in Part III-A, ASTM Standards for 1946. We have employed gasoline in this determination since it is representative of an important class of industrial products which are susceptible to deterioration, and for which it is important to provide stabilizing materials. The column headed IPI lists the Induction Period Increase, in minutes, over that of the gasoline in the absence of the antioxidants of our invention. That is, under the conditions of test, each gasoline exhibits a period, typical of the gasoline, wherein oxygen is not absorbed. In the presence of our inhibitors this period is increased by the amount listed under IPI. The lack of effectiveness of N-(p-hydroxyphenyl)urea is shown by compound No. 8 in the table.

Table

EFFECT ON INDUCTION PERIOD INCREASE OF GASOLINE

| No. | Additive                                | IPI, Min. |
|-----|-----------------------------------------|-----------|
| 1   | N-(mixed amyl)-N'-(p-hydroxyphenyl)urea | 755       |
| 2   | N-n-octyl-N'-(p-hydroxyphenyl)urea      | 520       |
| 3   | N-n-dodecyl-N'-(p-hydroxyphenyl)urea    | 485       |
| 4   | N-n-propyl-N'-(p-hydroxyphenyl)urea     | 395       |
| 5   | N-cyclohexyl-N'-(p-hydroxyphenyl)urea   | 390       |
| 6   | N-n-butyl-N'-(p-hydroxyphenyl)urea      | 255       |
| 7   | N-n-octadecyl-N'-(p-hydroxyphenyl)urea  | 195       |
| 8   | N-(p-hydroxyphenyl)urea                 | 25        |

We have disclosed a number of embodiments of our invention and illustrated several methods whereby these materials can be prepared. However, our invention is not intended to be limited to the specific examples herein or to the means

described herein for obtaining our novel compounds.

We claim:

1. A new petroleum hydrocarbon fuel composition stable to oxidation consisting essentially of gasoline, normally susceptible to deterioration by oxygen and, in amount sufficient to prevent such deterioration, an antioxidant material consisting of an N'-(p-hydroxyphenyl)urea substituted on the N-nitrogen atom with a member selected from a group consisting of acyclic and cyclic saturated paraffin radicals containing up to about 18 carbon atoms.
2. A new petroleum hydrocarbon fuel composition stable to oxidation consisting essentially of gasoline, normally susceptible to deterioration by oxygen and, in amount sufficient to prevent such deterioration, an antioxidant material consisting of an N'-(p-hydroxyphenyl)-urea substituted on the N-nitrogen atom with an acyclic saturated paraffin radical containing up to about 18 carbon atoms.
3. A new petroleum hydrocarbon fuel composition stable to oxidation consisting essentially of gasoline, normally susceptible to deterioration by oxygen and, in amount sufficient to prevent such deterioration, an antioxidant material consisting of an N'-(p-hydroxyphenyl)-urea substituted on the N-nitrogen atom with a cyclic saturated paraffin radical containing up to about 18 carbon atoms.
4. A new petroleum hydrocarbon fuel composition stable to oxidation consisting essentially of gasoline, normally susceptible to deterioration by oxygen and, in amount sufficient to prevent such deterioration, an antioxidant material consisting of N-cyclohexyl-N'-(p-hydroxyphenyl)-urea.
5. A new petroleum hydrocarbon fuel composition stable to oxidation consisting essentially of gasoline, normally susceptible to deterioration by oxygen and, in amount sufficient to prevent such deterioration, an antioxidant material consisting of N-n-propyl-N'-(p-hydroxyphenyl)-urea.
6. A new petroleum hydrocarbon fuel composition stable to oxidation consisting essentially of gasoline, normally susceptible to deterioration by oxygen and, in amount sufficient to prevent such deterioration, an antioxidant material consisting of N-(mixed-amyl)-N'-(p-hydroxyphenyl)-urea.
7. A new petroleum hydrocarbon fuel composition stable to oxidation consisting essentially of gasoline, normally susceptible to deterioration by oxygen and, in amount sufficient to prevent such deterioration, an antioxidant material consisting of N-n-octyl-N'-(p-hydroxyphenyl)-urea.
8. A new petroleum hydrocarbon fuel composition stable to oxidation consisting essentially of gasoline, normally susceptible to deterioration by oxygen and, in amount sufficient to prevent such deterioration, an antioxidant material consisting of N-n-dodecyl-N'-(p-hydroxyphenyl)-urea.

References Cited in the file of this patent

#### UNITED STATES PATENTS

| Number    | Name    | Date          |
|-----------|---------|---------------|
| 2,266,601 | Howland | Dec. 16, 1941 |
| 2,477,872 | Haury   | Aug. 2, 1949  |